

## UNITED STATES PATENT OFFICE

BROB NATANAEL SEGERFELT, OF BOHMISCH KRUMAU, CZECHOSLOVAKIA

## METHOD OF PRODUCING CELLULOSE

No Drawing. Application filed April 21, 1928, Serial No. 271,985, and in Sweden April 23, 1927.

In the production of cellulose by boiling cellulosic substances with acid or alkaline digester liquor and afterwards washing the cellulose obtained in diffusers or similar 5 washing apparatus, it has hitherto been common practice to use the strongest waste or black liquor obtained from the diffusers or other washing apparatus for the regeneration of fresh digester liquor or white liquor 10 and consequently, there only remained waste liquor of a weaker concentration available for the purpose of adding to the white liquor in order to make up the required volume of total liquor in the digester. The washing of 15 the pulp in the diffusers was performed in such manner that the waste liquor drawn from one diffuser being washed with hot water, was not passed over to the top of a second newly blown diffuser to serve as a primary 20 wash in the same, until the concentration of the waste liquor from the first diffuser had decreased to a specific gravity of 1.074, or even lower. By using a weak black liquor to make up the required volume of total liquor 25 in the digester and as a primary wash in a newly blown diffuser the black liquor obtained from such diffuser for the regeneration of white liquor will only have a concentration not exceeding 1.107, and consequently, 30 large quantities of water must be evaporated from the same. The regenerated soda has as a rule been dissolved in molten state in water or in a weak NaOH-solution, but since the degree of causticizing decreases at a high 35 concentration of the soda solution, it is common practice not to make the soda solution of a higher concentration than of a specific gravity of 1.179, and therefore, when such soda solution is causticized, the white liquor 40 obtained will have a low concentration, and this liquor when used in the digester will give a weak black liquor.

The present invention has for its purpose to render it possible to obtain from the diffusers, or other washing apparatus, a waste

liquor of a higher concentration than that hitherto obtained, so that the volume of black liquor to be regenerated per unit weight of cellulose produced will be decreased, and consequently the cost of recovery of the chemicals reduced. One feature of the present 50 method consists in that the strongest black liquor obtained from the diffusers or other washing apparatus used, is utilized as supplemental liquor added to the fresh white liquor to make up the required volume of total liquor for a subsequent cook. From this cook a waste liquor will thus be obtained which has a higher concentration than usual, and the strong waste liquor first drawn from 55 the diffusers from this cook is used as supplemental liquor for the next cook. By proceeding in this manner practically any desired concentration of the waste liquor may be obtained. The waste liquor used as supplemental liquor should have a specific gravity 60 of at least 1.124. A further feature of the present method consists in that as a primary wash in a newly blown diffuser waste liquor drawn from another diffuser is used which, 65 when such washing is begun, has a comparatively high concentration, namely, a specific gravity of at least 1.090, whereby the waste liquor passing from such newly blown diffuser will be less diluted.

A further feature of the present method, as applied to the use of alkaline digester liquor, consists in that the soda obtained by the regeneration of the waste liquor, is dissolved in a strong NaOH-solution holding at least 70 50 kg. NaOH per cu. m., whereby it is possible to increase the concentration of the resulting solution, i. e., the green liquor, since the same quantity of sodium carbonate may be dissolved as when water or a weak NaOH-solution is used, without the quantity of lime to be added for causticizing having to be increased. The white liquor thus prepared will 75 therefore contain more NaOH per cubic meter 80 than is now usual, and consequently, a less 85 90

volume of water for the total active alkali used per charge. Therefore, a correspondingly greater volume of strong black liquor obtained in the manner above stated, can be 6 added to the white liquor to make up the required volume of total liquor, which will aid to give a high concentration of the waste liquor resulting from the cook.

In order to make the present method more 10 easily understood, a manner in which it may be carried out in practice will now be described.

A vertical digester for sulphate cellulose is charged with 10000 kg. wood chips, holding 15 2500 kg. water, after which fresh digester liquor, termed white liquor here below, is added, said liquor being assumed to have a specific gravity of 1.142 and consisting of NaOH, Na<sub>2</sub>S and some Na<sub>2</sub>CO<sub>3</sub>, in such quantities that the active alkali, i. e. NaOH and Na<sub>2</sub>S, amounts to 1400 kg. Assuming that the strength of the white liquor is 120 kg. active alkali per cu. m., 11.7 cu. m. white liquor is thus required. This quantity of liquor 20 25 is too small, however, to effect the circulation required for the digestion, and for this reason waste liquor from a preceding digestion, termed black liquor here below, must be added. In this case 13.9 cu. m. of such black liquor having an assumed specific gravity of 1.107, are added. The total 30 35 quantity of liquor, including the water in the wood, thus becomes 28.1 cu. m.

Now, the invention has for its purpose by 35 various steps in the process of manufacture to concentrate the black liquor obtained from the digester and which is to be regenerated. One step consists in removing water from the digester liquor during the digestion, either 40 by means of powerful gassing off, or by evaporation of the digester liquor in special apparatus connected to the digester. By gassing off it should be possible, in the present case, to remove 1200 kg. water from the digester. 45 In the remaining digester liquor lignin etc. is dissolved from the wood during the digestion, so that, in the case assumed, the black liquor may be assumed to have a specific gravity of 1.149 at the end of the digestion. When 50 the digestion is finished, the pulp and the black liquor are blown at a pressure of from 3 to 4 kg. from the digester to a diffusor, or similar washing apparatus, in order to wash the cellulose obtained clear from the black 55 liquor. A newly blown diffusor is first washed with a weak liquor from another previously blown diffusor, whereby the strong black liquor in the first diffusor becomes less diluted, than if the diffusor were first 60 washed with clean water. From the newly blown diffusor a strong black liquor is obtained at the beginning of the washing, which liquor by prior practice has been always sent to the soda house for regeneration of alkali, 65 but according to the present invention such

strong black liquor is used in the first place as supplemental liquor for a new charge in the digester. Such liquor should not have a lower specific gravity than 1.124. Instead of using, as such supplemental liquor, a black 70 liquor having a specific gravity of 1.107, for instance, as has heretofore been customary, the strongest black liquor is thus used, which, in the case assumed, had a specific gravity of 1.149. In this manner a black liquor is 75 obtained from the second boiling, which has a specific gravity of 1.160. This liquor is used in the first place as a supplemental liquor for charging a third boiler, which thus gives a still stronger waste liquor having a specific 80 gravity of 1.170. This course is proceeded with until the desired concentration of the black liquor is obtained. Furthermore, by washing over from one diffusor to another, as above described, the newly blown diffusor 85 is commenced at a higher concentration of the waste liquor than that hitherto used, namely, with black liquor having at the outset a specific gravity not lower than 1.090, the region of dilution becomes more limited 90 during the washing, and accordingly the black liquor less diluted. In this manner it is possible for the regeneration to obtain a liquor having practically any desired concentration. In practice, however, it is not 95 suitable to go beyond the point where the liquor remains liquid at 30° C., that is to say, it should not congeal at this temperature. That portion of the strong black liquor obtained in the manner above described which 100 is not needed as supplemental liquor for the next digestion, is further evaporated, if required, in suitable evaporation apparatus, or is directly combusted in suitable combustion apparatus.

By using white liquor having a higher percentage of alkali, such as, for instance, 180 kg. active alkali per cu. m., only 7.8 cu. m. white liquor is needed in the case above assumed, instead of 11.7 cu. m., and for this reason it 105 will thus be possible to replace 3.9 cu. m. water with concentrated black liquor, which will further contribute to increasing the concentration of the black liquor. This, however, it has previously not been possible to do in 110 practice, for the reason that the degree of causticizing decreases at a high concentration of the soda solution to be causticized. It is usual to prepare the white liquor in such manner that the evaporated soda is dissolved 115 in a melting state in water or in a weak white liquor obtained from washing the calcium carbonate precipitate obtained in the causticizing of the soda. Now, if this soda solution is made of a too high concentration it becomes difficult to causticize a high percentage of the sodium carbonate present in the solution. According to the present invention this difficulty is avoided by dissolving the melting 120 soda in a strong solution of white liquor, 125

holding at least 50 kg. NaOH per cu. m., whereby the concentration of the solution as far as the quantity of NaOH in the same is concerned, will of course be increased with-  
 5 out the quantity of sodium carbonate in the solution exceeding that quantity which is suitable for obtaining a high degree of causticizing.

The advantages of the present method will  
 10 be readily appreciated by those skilled in the art. With the use of the present method it is possible, without procuring new apparatus, in a soda or sulphate cellulose plant to obtain a black liquor for the soda house having  
 15 such specific gravity that only 4.5 cu. m. black liquor per 1000 kg. cellulose will have to be evaporated.

I claim:

1. The method of producing cellulose  
 20 which comprises digesting cellulosic material with digester liquor and afterwards washing the cellulose produced in diffusors, evaporating the strongest waste liquor obtained from the diffusors from a previous boiling, and  
 25 adding such evaporated waste liquor as supplemental liquor to the fresh digester liquor for obtaining the required quantity of liquid in the digester.

2. The method of producing cellulose  
 30 which comprises digesting cellulosic material with digester liquor and afterwards washing the cellulose produced in diffusors, performing the first washing in said diffusors with waste liquor having at the outset a specific  
 35 gravity not less than 1.090, and adding the strongest waste liquor obtained from such washing in said diffusors as supplemental liquor to the fresh digester liquor for obtaining the required quantity of liquid in the  
 40 digester.

3. The method of producing cellulose which comprises digesting cellulosic material with digester liquor in a digester, concentrating the digester liquor in the digester during  
 45 the digestion by removing steam from the same, blowing the pulp and liquor to diffusors when the digestion is completed, performing the first washing in said diffusors with waste liquor having at the outset a specific  
 50 gravity not less than 1.090, and using the strongest waste liquor first obtained from such washing in said diffusors as supplemental liquor to the fresh digester liquor introduced into the digester for a subsequent digestion of a new charge.

4. The method of producing cellulose which comprises digesting cellulosic material with alkaline digester liquor in a digester, concentrating the digester liquor in the digester during the digestion by removing steam from the same, blowing the pulp and liquor to diffusors when the digestion is completed, performing the first washing in said diffusors with waste liquor having at the outset a specific gravity not less than 1.090, and

using the strongest waste liquor obtained from such washing in said diffusors as supplemental liquor to the fresh digester liquor introduced into the digester for a subsequent digestion of a new charge, regenerating the remaining portion of the waste liquor to produce soda therefrom, dissolving such soda in a strong NaOH-solution, and causticizing such solution to produce fresh digester liquor.

BROR NATANAEL SEGERFELT.